

Aug. 29, 1944.

R. H. LOMBARD

2,356,937

VITRIFIED DIAMOND GRINDING WHEEL

Filed May 10, 1941



FIG. 1



FIG. 2



FIG. 3



FIG. 4



FIG. 5

Inventor

ROBERT H. LOMBARD

By Gen. Geom. Stripp  
Attorney

## UNITED STATES PATENT OFFICE

2,356,937

## VITRIFIED DIAMOND GRINDING WHEEL

Robert H. Lombard, Worcester, Mass., assignor  
to Norton Company, Worcester, Mass., a cor-  
poration of Massachusetts

Application May 10, 1941, Serial No. 392,829

9 Claims. (Cl. 51—307)

The invention relates to vitrified diamond grinding wheels.

One object of the invention is to provide improved structures for vitrified bonded diamond grinding wheels and sticks or hones which shall be simple to produce, reliably controllable in processing so as to achieve uniformity of structures in quantity production, and give consistently good results structural and functional. Another object of the invention is to provide a structure for two-part vitrified diamond grinding wheels having an abrasive rim or periphery and a non-abrasive center, which structure shall be integral and can be duplicated with few, if any, rejections during manufacture. Another object of the invention is to provide abrasive articles of the above-mentioned kind with highly advantageous mechanical or physical structural elements internally and at the same time, during firing, to control and prevent swelling of either the center or the abrasive portion of a vitrified bonded diamond grinding wheel. Another object is to provide body materials to take part in building up, during firing, a compound framework usable either in the abrasive portion to provide improved support for the abrasive grains or in the backing or center for the abrasive portion to provide improved support for the latter, and capable of use in both the abrasive portion or in the backing or center, and in any such case to achieve the desired strength of structure while adequately accounting for the effects of thermal changes, during manufacture, or during use, within the article. Another object is to provide body materials well adapted for conjoint use and coaction in the carrying out of this last-mentioned object. Another object of the invention is to provide a mix for a center for such a wheel capable of being matured into a strong and uniform center in a vitrifying process. Other objects will be in part obvious or in part pointed out hereinafter.

The invention accordingly consists in the features of construction, combinations of elements, arrangements of parts, and in the several steps and relation and order of each of said steps to one or more of the others thereof, all as will be illustratively described herein, and the scope of the application of which will be indicated in the following claims.

In the accompanying drawing illustrating one of many possible embodiments of the mechanical features of this invention,

Figure 1 is a cross sectional view of a mold having just been filled with a vitrifiable non-

abrasive mix to form the center of a peripheral vitrified diamond grinding wheel;

Figure 2 shows the mold of Figure 1 with a top plate in position;

Figure 3 shows the mold of Figures 1 and 2 after pressing of the center, after inversion, after the mold ring has been removed and a two-diameter mold band placed outside of the largest mold plate;

Figure 4 shows the mold in the same condition as in Figure 3 after the annular space has been filled with diamond ceramic material and the ring reinserted; and

Figure 5 shows the mold of Figure 4 after it is closed.

The drawing illustrates the manufacture of a peripheral wheel. From this it should not be understood that peripheral wheels are more important or manufactured in greater quantities than cup wheels and others having an annular plane abrasive surface because perhaps the reverse is the fact, but the manufacture of a peripheral ceramic diamond grinding wheel presents particular problems and from the following disclosure the manufacture of a diamond ceramic cup wheel will be readily understood. In the first place, it may be noted that owing to the great cost of diamonds, it is quite usual to make diamond grinding wheels in the form of a thin annulus of diamond abrasive with a non-abrasive center. A ceramic bonded diamond abrasive wheel has certain free-cutting and wear resisting properties which make it highly desirable for certain grinding operations. It is desirable to make a vitrified center for such diamond grinding wheels and in order to make an integral body free from cracks or strains, it is desirable to vitrify the center or back at the same time that the rim is vitrified.

Swelling is a particular problem and, therefore, it is important to provide a mix both for the center and the annulus which will not swell during firing. To prevent the development of strains or cracks in the product, it is important that the annulus and the center be consolidated into a single piece of uniform density. I shall first describe the steps in the molding technique for the production of a green body ready for firing in a suitable furnace.

Referring now to Figure 1, I provide a large flat plate 8 and a mold consisting of a plate 10, a ring 11, and an arbor 12. The ring 11 just fits the plate 10 and the arbor 12 just fits in a central hole 13 in the plate 10. I first place the plate 10 upon the plate 8 and at opposite sides

of the plate 10 I position a pair of spacing blocks 14. I then place the ring 11 around the plate 10 and upon the blocks 14, as shown. I then insert the arbor 12 part way into the hole 13. I now fill the mold with a center non-abrasive mix 15 and level it off in a well known manner.

I now transfer the filled mold of Figure 1 on the plate 9 to the bottom plate of a hydraulic press. Referring to Figure 2, I now place upon the arbor 12 a plate 16 having an arbor hole 17 and having a diameter somewhat greater than that of the plate 10. I now remove the blocks 14 and temporarily hold up the ring 11 with my fingers. Then I apply the pressure of the hydraulic press to the extent of about 250 pounds per square inch. After the ring 11 starts to move, sufficient grit moves between it and the plate 10 to prevent the ring 11 from dropping.

I now strip the mold ring 11 and invert the mold, locating the plate 16 on the bottom plate of the hydraulic press. A consolidated center mix 15a is now located between the plates 10 and 16. Then I place a heavy mold band 18 around the plate 16 and upon spacing blocks 19. The mold band 18 has a small inside diameter approximately the same as that of the outside diameter of the plate 16 so as to fit upon it with a sliding fit. It has a larger inside diameter separated therefrom by a shoulder 21. When the band 18 is raised by the blocks 19, the shoulder 21 is somewhere between the top and bottom of the plate 10.

This leaves a space 22 bounded on the bottom by the plate 16, on the outside by the mold band 18, and on the inside by the periphery of the plate 10 and the periphery of the consolidated center 15a. The top of this space 22 to be filled is somewhat below the level of the shoulder 21. Referring to Figure 4, I now fill this space with a diamond containing ceramic mix 23. I then place the ring 11 inside the mold band 18 upon the shoulder 21, as shown. It will be noted that the height of the ring 11 is the same as that of the plate 10 but the distance from the shoulder 21 to the top of the mold band 18 is slightly less. I now remove the spacing blocks 19 and close the mold to the position shown in Figure 5. The quantity of material 15 and 23, respectively, is selected so that the two parts of the wheel will be pressed to definite, predetermined densities or packings of their constituents, and usually so that the two parts of the wheel will have similar densities of packing, that is, the porosity of the rim and the center will be similar. The closing of the mold to the position shown in Figure 5, however, further presses the consolidated mix 15a simultaneously with the compression of the fill 23, so that the pressed center 15b and the pressed fill 23a are of equal height and consolidated into an integral article which can be readily handled even before it is fired. Such an article is termed a "green" wheel in the abrasive industry.

I now strip the mold band 18, remove the plug 12, and then pick off the plate 16 and the plate 10 and ring 11. I now have a "green" wheel consisting of a non-abrasive center part 15b and an abrasive periphery 23a in an integral piece, with ceramic material throughout capable of being fired in a suitable furnace into an integral non-swelled grinding wheel.

Considering now the materials which I use to form the abrasive periphery 23a and the center or backing 15b, the former contains diamonds while the latter does not; both parts include

ceramic materials, and in accordance with the present invention one or both of the parts contains silicon, or silicon alloy, such as ferro-silicon or aluminum-silicon, all of which are generically referred to herein as metallic silicon, or sometimes as oxidizable metallic silicon. The use of silicon, in accordance with the manner in which I employ it, has at least two desirable functions: (1) It functions during firing to prevent detrimental swelling of the abrasive body due to the evolution of certain gases from the material during the burn in a non-oxidizing atmosphere, and (2) since I insure its presence as granular silicon in the final fired article, I cause the silicon to provide at the same time suitable solid granular material for that strongly vitrified bonded framework of the abrasive body which is essential to the achievement of certain practical advantages such as mechanically strong and adequate support of the diamond grains and consequent low wear during grinding. This use and functioning of silicon has enabled me to make non-swelled diamond containing abrasive bodies of excellent quality bonded with a vitrified bond matured in the vicinity of 1000° C. or below in a non-oxidizing atmosphere.

Silicon of various grit sizes may be used. For example, a grit size may be chosen which confers the greatest bonded strength on the diamond grains in the abrasive body or wheel. In this connection fairly fine grit sizes seem to be more effective. I have used silicon of grit size through 100 mesh screen onto 210 mesh screen; silicon which has passed 210 mesh screen; and ball-milled silicon which is the finest of these grit sizes.

Examples of the calculated compositions for the abrasive periphery involving the use of silicon are:

|                               | Example 1 | Example 2 |
|-------------------------------|-----------|-----------|
|                               | Vol. %    | Vol. %    |
| 45 Diamond, 100 grit size     | 25        | 25        |
| Silicon, through 100 onto 210 | 25        | 25        |
| Silicon, through 210          |           |           |
| Bond A                        | 35        | 35        |
| Pores                         | 15        | 15        |

50 Bond A consists of 25 parts of ball clay, 2 parts of aluminum powder, and 75 parts of a frit according to the following formula, all parts being by weight:

|                    | Parts |
|--------------------|-------|
| Borax              | 32.2  |
| Boric acid         | 25.4  |
| Silica             | 37.6  |
| Hydrate of alumina | 1.0   |
| Whiting            | 3.8   |

60 The calculated chemical composition of this frit is as follows:

|                                   | Per cent |
|-----------------------------------|----------|
| Na <sub>2</sub> O                 | 7.3      |
| CaO                               | 3.       |
| 65 Al <sub>2</sub> O <sub>3</sub> | 9        |
| B <sub>2</sub> O <sub>3</sub>     | 36.4     |
| SiO <sub>2</sub>                  | 52.4     |

70 These wheels were burned at 950° C. for four and one-half hours in a non-oxidizing atmosphere of nitrogen.

If silicon is used for only part of the "body material" of a diamond containing abrasive body, it should be present at least in a proportion great enough to control the swelling which might otherwise occur during the burn in a non-

oxidizing atmosphere. The materials which constitute the remainder of the granular body material should have no harmful effect on the intended diamond abrasive body; they should not be deleteriously affected by the bond or the burning conditions; they should have no deleterious effect on the diamond abrasive; they should contribute satisfactorily to the bonded strength of the diamond abrasive body, and they should have a coefficient of thermal expansion which causes neither deleterious cracking of the vitrified bond nor undesirable stresses in the abrasive body. For example, I have used vitreous silica as such substance mixed with silicon to form the body material of vitrified bonded diamond abrasive bodies, and examples of such compositions are given below.

The above use of silicon as a body material in a diamond containing abrasive body burned in a non-oxidizing atmosphere is to be considered as a specific application of a general principle, namely, the use as body material in a vitrified bonded, diamond containing abrasive body of a substance or substances which (1) by virtue of their reducing nature or other properties are capable of preventing or controlling the swelling caused by gas evolution from the materials during a burn in a non-oxidizing atmosphere, (2) are proportioned in an amount at least great enough to prevent or control such swelling, and (3) in addition to their qualities of preventing swelling are also present in form and amount to be capable of forming, in whole or in part, the granular material of a vitrified bonded framework which affords a suitable strong, wear-resistant support to the diamond grains of the diamond abrasive body. Other illustrative substances which may be used for this purpose are ferro-silicon and silicon-aluminum alloys.

My invention further involves the use of granular silicon as a solid constituent or body material of a vitrified bonded body, such as the center 15b integrally bonded to and used as a support for a vitrified bonded diamond containing abrasive body, such as the peripheral rim 21a of a vitrified bonded diamond grinding wheel.

A central supporting center made solely of granular vitreous silica, bonded by a vitreous bond such as bond A is apt to swell objectionably when burned in a non-oxidizing atmosphere due to the evolution of gas from its constituent materials. This swelling may seriously disturb the structure of portions of the peripheral diamond containing rim which are adjacent to the supporting center. The use of two parts of aluminum powder in the bond diminishes this swelling, but not always sufficiently. I have found that the use of granular silicon as the whole or part of the granular constituents of the central supporting disk or backing obviates this swelling satisfactorily, and at the same time the silicon provides a suitable material for the vitrified bonded framework of the supporting center. Here also, as in the diamond containing rim, the silicon grain serves the dual function of controlling the swelling in a non-oxidizing atmosphere and of serving as a structural element of the center in that, as in the abrasive-containing rim, the silicon is present in the final or fired product, exclusive of any oxidation product formed by part or some of it during firing in the process of controlling swelling, in the form of individual grain-like entities or metallic granules distributed throughout and bonded by the

now-vitrified bond to form a structural part of a compound framework. In the sense that some of the initially present metallic silicon is oxidized during firing to prevent swelling and hence produces some oxidation product, it may be said that the silicon present in the final vitrified article to take part in forming this compound framework is preponderantly metallic silicon or silicon per se to distinguish it from any such oxidation product which, in contrast, goes into solution in the molten bond glass during firing. Again, silicon is to be considered only as a specific example of substances which make possible attaining the above effects.

The principles governing the range of grit sizes of the granular material for the vitrified bonded supporting center are different from those for the diamond containing abrasive body. For the supporting center there is no need to select the grit size with a view to contributing maximum bonding support to the diamond abrasive grains of a particular grit size. As far as strength is concerned it is sufficient to provide a supporting center which will endure the mechanical stresses of the grinding operation without danger of breakage and yet be soft enough to be easily trued. Very fine grit material, such as has been ball milled finer than 210 grit size, is usually to be avoided in the supporting centers because it favors springback and the formation of pressure cracks during molding and it also favors shrinkage during the burning. However, fairly fine material, for example, through 100 mesh onto 210 mesh screen is desirable in the supporting center because it will nullify a tendency, present with coarse grained material, for cracks to form in the bond glass as a result of differential expansion between vitrified bond and the grains of the body material. Relatively fine grit material also makes it easier to produce well finished sides by the process of siding by grinding.

Mixtures of silicon with other suitable solid granular substances can be used as the body material for the vitrified bonded supporting center. I have used vitreous silica for such admixed material. In any event the material of the supporting center should be so chosen and proportioned that a difference in thermal expansion between the center and the peripheral diamond containing abrasive rim does not cause cracking or breaking of the rim or center. Also, the expansion of the body materials should match that of the bond sufficiently well to prevent cracking of the bond.

The vitrified ceramic bond of the supporting center or back can to advantage be of a less strongly bonding type than the vitrified bond in the diamond abrasive portion of the wheel or implement. Also, the percentage by volume of bond in the center or back can to advantage be less than in the diamond abrasive portion. If the strong bond and the high volume percentage of bond of the diamond abrasive portion is used in the non-abrasive center or back, the latter will be so hard that it will be unnecessarily difficult to true it, and there will be danger of breaking the product during truing. Therefore, I use a weaker bond in the non-abrasive center or back, for example, one which contains more clay; and I decrease the volume percentage of bond in the center in relation to that in the diamond abrasive portion. The weaker bonding of the supporting center or back thus attained facilitates truing and lessens the probability of crack-

ing during truing but, of course, the product retains adequate mechanical strength for the grinding operation. The above features of weakened bond composition and lessened bond proportion of the non-abrasive center are of real practical value because the supporting center may contribute by far a greater proportion of the surface to be trued than does the thin diamond abrasive rim.

Below are given by way of example compositions of vitrified bonded diamond wheels which I have made containing silicon in the diamond containing rim and in the non-diamond containing supporting center. This silicon serves the dual purpose described in the invention of preventing deleterious swelling during the burn in a non-oxidizing atmosphere, and of serving as a vitrified bonded granular structural element of the rim and the center. These wheels were 7 x  $\frac{1}{4}$  x  $1\frac{1}{4}$ " with a  $\frac{1}{8}$ " thick diamond containing rim.

In the wheel of Example 3 the body material of the rim and center was all silicon. In the wheel of Example 4 the body material was a mixture of silicon and vitreous silica, proportioned alike both in the rim and the center so as to avoid detrimental differential expansion between them.

*Vitrified bonded diamond containing abrasive wheels 7 x  $\frac{1}{4}$  x  $1\frac{1}{4}$ "*

|                                                    | Example 3                                    |                   | Example 4                                    |                   |
|----------------------------------------------------|----------------------------------------------|-------------------|----------------------------------------------|-------------------|
|                                                    | Diamond-containing rim $\frac{1}{8}$ " thick | Supporting center | Diamond-containing rim $\frac{1}{8}$ " thick | Supporting center |
| Diamond, 100 grit size.                            | Vol. % 25                                    | Vol. % 25         | Vol. % 25                                    | Vol. % 15         |
| Silicon, ball milled.                              |                                              |                   |                                              |                   |
| Silicon, through 100 onto 210 mesh screen.         |                                              | 65                |                                              | 30                |
| Vitreous silica, ball milled.                      |                                              |                   | 10                                           |                   |
| Vitreous silica, through 100 onto 210 mesh screen. |                                              |                   |                                              | 20                |
| Bond A.                                            | 35                                           |                   | 35                                           |                   |
| Bond B.                                            | 15                                           | 20                | 15                                           | 20                |
| Pores.                                             |                                              |                   |                                              | 15                |

Bond B consists of 35 parts of ball clay and 65 parts of the frit of bond A with two parts of aluminum powder and it is a weaker bond than bond A by virtue of its greater clay content.

The wheels of Examples 3 and 4 were excellent mechanically, were strong integral structures, and gave excellent results in grinding cemented carbides. They are especially free-cutting as compared with metal bonded diamond grinding wheels.

Although so far as certain features of the invention are concerned it is embodied in a grinding wheel, nevertheless certain advantages of the invention can be obtained when it is embodied in other types of abrasive articles such as honing sticks, abrasive stones, inserts, segments, and the like.

It will thus be seen that there has been provided by this invention an article of manufacture and a method in which the various objects hereinabove set forth together with many thoroughly practical advantages are successfully achieved. As various possible embodiments might be made of the mechanical features of the above invention and as the art herein described might be varied in various parts, all without departing from the scope of the invention, it is to be un-

derstood that all matter hereinbefore set forth or shown in the accompanying drawing is to be interpreted as illustrative and not in a limiting sense.

I claim:

1. A vitrified-bonded abrasive article comprising the bonded reaction product, as a result of firing, of a mix that comprises abrasive grains, metallic granules of metallic silicon, and vitrifiable bond, the metallic granules being present in the product in an amount, exclusive of any oxidation product formed during firing, to constitute substantially 15% by volume, or more, of the volume of the vitrified-bonded article and being bonded by and distributed throughout the vitrified bond thereby to reinforce the bond and to form with the vitrified bond a compound framework of metallic granules and vitrified bond material, of which the metallic granules are material structural parts, said abrasive grains being distributed throughout and supported by said compound framework and bonded therein by the vitrified bond of said framework.

2. A vitrified-bonded abrasive article having a unitary body comprising a vitrified-bonded abrasive layer and a vitrified-bonded backing layer, and being the unitary bonded reaction product as a result of firing together the two layers, one of which comprises abrasive grains, metallic granules preponderantly of metallic silicon, and vitrifiable bond, and the other of which comprises vitrifiable bond and metallic granules preponderantly of metallic silicon, said metallic granules being present in the vitrified abrasive layer in an amount, exclusive of any oxidation product formed during firing, to constitute substantially 15% by volume, or more, of the volume of the vitrified abrasive layer and being bonded by and distributed in said amount throughout the vitrified bond of said abrasive layer thereby to reinforce the bond and to form with it a compound framework of which the said metallic granules in said amount are material structural parts, said abrasive grains being distributed throughout and supported by said compound framework, and bonded therein by the vitrified bond, and said metallic granules being present in the vitrified-bonded backing layer in an amount, exclusive of any oxidation product formed during firing, to constitute substantially 40% by volume, or more, of the volume of the vitrified backing layer and being bonded by and distributed in said amount throughout the vitrified bond of said vitrified backing layer to form a compound framework of which the said metallic granules are material structural parts thereby to constitute said backing layer to support said vitrified-bonded abrasive layer.

3. A vitrified-bonded abrasive article comprising the bonded reaction product, as a result of firing, of a mix that comprises abrasive grains, metallic granules of metallic silicon, and vitrifiable bond, the metallic granules being present in the product in an amount, exclusive of any oxidation product formed during firing, to constitute substantially 15% by volume, or more, of the volume of the vitrified-bonded article and being bonded by and distributed throughout the vitrified bond thereby to reinforce the bond and to form with the vitrified bond a compound framework of metallic granules and vitrified bond material, of which the metallic granules are material structural parts, said vitrified bond being present in an amount to constitute on the order of 35% by volume of the fired article and said

abrasive grains being present in an amount to constitute on the order of 25% by volume of the fired article and being distributed throughout and supported by said compound framework and bonded therein by the vitrified bond of said framework.

4. A vitrified-bonded abrasive article comprising the bonded reaction product, as a result of firing, of a mix that comprises abrasive grains, vitrifiable bond, and body material comprising metallic granules of metallic silicon and granules of vitreous silica, the metallic granules being present in the product in an amount, exclusive of any oxidation product formed during firing, to constitute a substantial proportion of the volume of the vitrified-bonded article and the vitreous silica granules being present in an amount to constitute a material proportion of the volume of the vitrified bonded article, both said metallic granules and said vitreous silica granules being bonded by and distributed throughout the vitrified bond thereby to reinforce the bond and to form with the vitrified bond a compound framework of which both said metallic granules and said vitreous silica granules are material structural parts, said abrasive grains being distributed throughout and supported by said compound framework and bonded therein by the vitrified bond of said framework.

5. A vitrified-bonded abrasive article having a unitary body comprising a vitrified-bonded abrasive layer and a vitrified-bonded backing layer and being the unitary bonded reaction product as a result of firing together the two layers, one of which comprises abrasive grains, metallic granules of metallic silicon, and vitrifiable bond, and the other of which comprises vitrifiable bond, metallic granules of metallic silicon, and body material comprising granules of vitreous silica, the metallic granules being present in the vitrified abrasive layer in an amount, exclusive of any oxidation product formed during firing, to constitute a substantial proportion of the volume of the vitrified abrasive layer and being bonded by and distributed throughout the vitrified bond thereby to reinforce the bond and to form with the vitrified bond a compound framework of metallic granules and vitrified bond material, of which the metallic granules are material structural parts, said abrasive grains being distributed throughout and supported by said compound framework and bonded therein by the vitrified bond of said framework, said granules of vitreous silica being present in the vitrified-bonded backing layer in an amount to constitute a material proportion of the volume thereof and being bonded by and distributed throughout the vitrified bond of said backing layer to form a compound framework of which said granules of vitreous silica are material structural parts, and said metallic silicon being present in an amount at least sufficient to prevent deleterious swelling of said backing layer during firing.

6. A vitrified-bonded abrasive article having a unitary body comprising a vitrified-bonded abrasive layer and a vitrified-bonded backing layer and being the unitary bonded reaction product as a result of firing together the two layers, one of which comprises abrasive grains, metallic granules of metallic silicon, and vitrifiable bond, and the other of which comprises vitrifiable bond, metallic granules of metallic silicon, and body material comprising granules of vitreous silica, the metallic granules being pres-

ent in the vitrified abrasive layer in an amount, exclusive of any oxidation product formed during firing, to constitute a substantial proportion of the volume of the vitrified abrasive layer and being bonded by and distributed throughout the vitrified bond thereby to reinforce the bond and to form with the vitrified bond a compound framework of metallic granules and vitrified bond material, of which the metallic granules are material structural parts, said abrasive grains being distributed throughout and supported by said compound framework and bonded therein by the vitrified bond of said framework, said metallic granules being present in the vitrified bonded backing layer in an amount, exclusive of any oxidation product formed during firing, and said granules of vitreous silica being present in the vitrified bonded backing layer in an amount, together to constitute a substantial proportion of the volume of the vitrified backing layer and both being distributed throughout the vitrified bond thereof thereby to reinforce the bond and to form with the vitrified bond a compound framework of both said granules and vitrified bond material, of which both said metallic granules and said vitreous silica granules are material structural body parts.

7. A vitrified-bonded abrasive article comprising the bonded reaction product, as a result of firing, of a mix that comprises abrasive grains, metallic granules of oxidizable metallic silicon, and vitrifiable bond, the metallic granules being present in the vitrified product in an amount, exclusive of any oxidation product formed during firing as a result of oxidation of some of said metallic silicon, to constitute a substantial proportion of the volume of the vitrified article and being bonded by, and distributed in said amount throughout, the vitrified bond thereby to reinforce the bond and to form with the vitrified bond a built-up compound framework of which the metallic granules of metallic silicon, in said substantial proportion, are material structural parts, said abrasive grains being distributed throughout and supported by said built-up framework and bonded therein by the vitrified bond of said framework.

8. A vitrified-bonded abrasive article having a unitary body comprising a vitrified bonded abrasive layer and a vitrified bonded backing layer, and being the unitary bonded reaction product as a result of firing together two mixes, one of which comprises abrasive grains and vitrifiable bond and the other of which comprises vitrifiable bond and metallic granules of oxidizable metallic silicon, the metallic granules being present in the vitrified-bonded backing layer in an amount, exclusive of any oxidation product formed during firing as a result of oxidation of some of said metallic silicon, to constitute a substantial proportion structurally of the said backing layer and the said metallic granules being bonded by, and distributed in said substantial proportion throughout, the vitrified bond of said backing layer to form a built-up compound framework of which said metallic granules are, in said substantial proportion, material structural parts to thereby constitute said backing layer to support said abrasive layer.

9. A vitrified-bonded abrasive article having a unitary body comprising a vitrified-bonded abrasive layer and a vitrified-bonded backing layer, and being the unitary bonded reaction product as a result of firing together two mixes, one of which comprises abrasive grains and vitri-

fiable bond and the other of which comprises  
vitrifiable bond and granules of an oxidizable  
metallic silicon and body material comprising  
granules of vitreous silica, granules of said oxi-  
dizable metallic silicon and granules of said  
vitreous silica being present in the vitrified-  
bonded backing layer in an amount, exclusive  
of any oxidation product formed during firing  
as a result of oxidation of some of said metallic  
silicon, to constitute a substantial proportion  
structurally of the said backing layer and the

5 said granules of oxidizable metallic silicon and  
the said granules of vitreous silica being bonded  
by, and distributed in said substantial propor-  
tion throughout, the vitrified bond of said back-  
ing layer to form a built-up framework of which  
10 said oxidizable metallic silicon granules and  
vitreous silica granules are in said amount ma-  
terial structural parts to thereby constitute said  
backing layer to support said abrasive layer.

ROBERT H. LOMBARD.